

# United States Patent Office

2,737,455  
Patented Mar. 6, 1956

1

2,737,455

## FERRITIC CREEP-RESISTING STEELS

Henry William Kirkby and Charles Sykes, Sheffield, England, assignors to Thos. Firth & John Brown Limited, Sheffield, England, a British company

No Drawing. Application April 1, 1953,  
Serial No. 346,255

5 Claims. (Cl. 75—126)

This invention comprises improvements relating to ferritic creep-resisting steels.

It is well known that the majority of creep-resisting steels (ferritic and austenitic) contain molybdenum and this element is generally regarded as an essential constituent in such materials. In ferritic creep-resisting steels, molybdenum is invariably present, e. g. carbon-molybdenum, chromium-molybdenum, molybdenum-vanadium, chromium-molybdenum-vanadium, and other special steels.

Molybdenum is known to be an alloying element of strategic importance and hitherto has been regarded as a metal vital to a country's economy in so far as alloy steels suitable for high temperature applications are concerned.

The present invention provides alloy compositions which, without entailing the use of molybdenum as an alloying constituent, have creep-resisting properties comparable with or superior to those of the known molybdenum-containing creep-resisting steels referred to above.

The alloys provided by the invention comprise the following range of composition:

|           |                            |          |    |
|-----------|----------------------------|----------|----|
| Carbon    | 0.02                       | to 0.15% | 15 |
| Silicon   | 0.05                       | to 1.0%  |    |
| Manganese | 0.05                       | to 2.0%  |    |
| Chromium  | 0.10                       | to 3.5%  |    |
| Vanadium  | 0.05                       | to 1.0%  |    |
| Titanium  | 0.05                       | to 0.40% |    |
| Boron     | 0.003                      | to 0.05% |    |
| Iron      | The substantial remainder. |          |    |

Nickel in a proportion up to 1% may optionally be included in the composition. Tungsten may also be present up to 2% and actually confers some improvement on the alloys in question. Tungsten is, however, another alloying element of high strategic value and it is to be noted that its inclusion in alloys of the present invention is not essential.

The preferred range of composition according to the invention is:

|           |       |          |    |
|-----------|-------|----------|----|
| Carbon    | 0.06  | to 0.12% | 55 |
| Silicon   | 0.10  | to 0.50% |    |
| Manganese | 0.50  | to 1.0%  |    |
| Chromium  | 0.40  | to 2.0%  |    |
| Vanadium  | 0.25  | to 0.75% |    |
| Titanium  | 0.075 | to 0.30% | 60 |

2

Boron-----0.003 to 0.01%.  
Iron-----Remainder.

The following stress rupture properties have been obtained on selected compositions within the range of the invention:

| 10 | Alloy | C, percent | Si, percent | Mn, percent | Ni, percent | Cr, percent | V, percent | Ti, percent | B, percent | Hours to Fracture under conditions, 14 tons/sq. inch at 600° C. |
|----|-------|------------|-------------|-------------|-------------|-------------|------------|-------------|------------|-----------------------------------------------------------------|
|    | A     | 0.05       | 0.65        | 0.74        | 0.05        | 0.64        | 0.43       | 0.08        | 0.005      | 163.                                                            |
|    | B     | 0.05       | 0.35        | 1.02        | nil         | 0.88        | 0.74       | 0.20        | 0.005      | 116 $\frac{1}{4}$ .                                             |
| 5  | C     | 0.04       | 0.31        | 0.94        | nil         | 0.64        | 0.51       | 0.24        | 0.01       | 300 Unbroken.                                                   |
|    | D     | 0.06       | 0.31        | 0.76        | nil         | 0.75        | 0.51       | 0.22        | 0.005      | 389.                                                            |
|    | E     | 0.07       | 0.35        | 0.96        | 0.07        | 3.19        | 1.0        | 0.14        | 0.005      | 306 Unbroken.                                                   |

On alloy A, a creep test under conditions 6 tons/sq. inch at 650° C. gave a creep deformation of 0.125% in 300 hours. This compares very favourably with the creep properties of known molybdenum-vanadium creep-resisting steels.

We claim:

1. A creep resistant ferritic alloy steel comprising carbon 0.02 to 0.15%, silicon 0.05 to 1.0%, manganese 0.05 to 2.0%, chromium 0.10 to 3.5%, vanadium 0.05 to 1.0%, titanium 0.05 to 0.40%, boron 0.003 to 0.05%, and the balance iron with impurities in ordinary amounts.
2. A creep resistant ferritic alloy steel comprising carbon 0.02 to 0.15%, silicon 0.05 to 1.0%, manganese 0.05 to 2.0%, chromium 0.10 to 3.5%, vanadium 0.05 to 1.0%, titanium 0.05 to 0.40%, boron 0.003 to 0.05%, nickel 0 to 1% and the balance iron with impurities in ordinary amounts.
3. A creep resistant ferritic alloy steel comprising carbon 0.06 to 0.12%, silicon 0.10 to 0.50%, manganese 0.50 to 1.0%, chromium 0.40 to 2.0%, vanadium 0.25 to 0.75%, titanium 0.075 to 0.30%, boron 0.003 to 0.01%, and the balance iron with impurities in ordinary amounts.
4. A creep resistant ferritic alloy steel comprising carbon 0.02 to 0.15%, silicon 0.05 to 1.0%, manganese 0.05 to 2.0%, chromium 0.10 to 3.5%, vanadium 0.05 to 1.0%, titanium 0.05 to 0.40%, boron 0.003 to 0.05%, and the balance iron with impurities in ordinary amounts, characterised by the total absence of molybdenum from the constituents.
5. A creep resistant ferritic alloy steel comprising carbon 0.02 to 0.15%, silicon 0.05 to 1.0%, manganese 0.05 to 2.0%, chromium 0.10 to 3.5%, vanadium 0.05 to 1.0%, titanium 0.05 to 0.40%, boron 0.003 to 0.05%, and the balance iron with impurities in ordinary amounts, characterised by the total absence of both molybdenum and tungsten from the constituents.

References Cited in the file of this patent

### UNITED STATES PATENTS

|           |              |               |
|-----------|--------------|---------------|
| 2,480,151 | Malcolm      | Aug. 30, 1949 |
| 2,542,220 | Urban et al. | Feb. 20, 1951 |
| 2,572,191 | Payson       | Oct. 23, 1951 |